

R. AUSTIN.  
Manufacture of Horseshoes.

No. 148,916.

Patented March 24, 1874.



Witnesses.  
George E. Uphaus,  
Robert Everett.

Inventor  
Richard Austin,  
Clipman, Austin & Co.,  
Atty.

# UNITED STATES PATENT OFFICE.

RICHARD AUSTIN, OF SING SING, NEW YORK.

## IMPROVEMENT IN THE MANUFACTURE OF HORSESHOES.

Specification forming part of Letters Patent No. 148,916, dated March 24, 1874; application filed January 24, 1874.

*To all whom it may concern:*

Be it known that I, RICHARD AUSTIN, of Sing Sing, in the county of Westchester and State of New York, have invented a new and valuable Improvement in the Manufacture of Horseshoes; and I do hereby declare that the following is a full, clear, and exact description of the construction and operation of the same, reference being had to the annexed drawings making a part of this specification, and to the letters and figures of reference marked thereon.

Figure 1 of the drawing is a representation of a bottom view of a horseshoe, showing my device. Fig. 2 is an end view of the same. Fig. 3 is a sectional view of the same.

This invention has relation to the manufacture of horseshoes; and it consists in first welding lugs of steel to the toe and heel portions of a shoe; then, after allowing these lugs to cool gradually, filing them so as to leave transverse grooves terminating in sharp edges; and then, as a final process, tempering the calks, as will be hereinafter explained.

The following is a description of my invention:

In the annexed drawings, A designates a horseshoe of the well-known form, and B B' B' are the toe and heel calks. These calks I make of steel, and arrange them as shown in

Fig. 1—that is to say, the calk is at right angles to the length of the shoe, and the heel-calks stand at an angle thereto.

I first weld to the sole of the shoe three oblong lugs or blanks, and allow them to cool slowly, so as to leave them soft and easily filed. I then file grooves into them in a direction with their length, and form sharp edges a a, with a deep groove between them. I finally temper the calks, and thus render them hard and durable.

Calks thus constructed and applied to shoes will take a very firm hold into ice or snow, and they are not liable to become detached under the roughest usage.

What I claim as new, and desire to secure by Letters Patent, is—

The method herein described of first attaching the calks to the shoe by welding; secondly, filing the calks to the shape substantially as shown and described, and then tempering them, as set forth.

In testimony that I claim the above I have hereunto subscribed my name in the presence of two witnesses.

RICHARD AUSTIN.

Witnesses:

HENRY C. NELSON,  
ISAAC B. NOXON.